

# UNITED STATES PATENT OFFICE.

MATTHEW GRAFF, OF PITTSBURG, PENNSYLVANIA.

## PROCESS OF MANUFACTURING STEEL DIRECT FROM THE ORE.

SPECIFICATION forming part of Letters Patent No. 393,553, dated November 27, 1888.

Application filed January 4, 1888. Serial No. 259,795. (No specimens.)

To all whom it may concern:

Be it known that I, MATTHEW GRAFF, a citizen of the United States, residing at Pittsburgh, in the county of Allegheny and State of Pennsylvania, have invented or discovered a certain new and useful Improvement in the Process of Manufacturing Steel Direct from the Ore, of which improvement the following is a specification.

10 In the attempts heretofore made to manufacture steel direct from the ore the carbonaceous material and the ore were crushed or broken up, and after being thoroughly mingled were placed in a suitable furnace and subjected 15 to a reducing-heat. This method, however, has proved practically unsuccessful on account of the rapid combustion of the carbonaceous material, which would be entirely consumed before thorough deoxidation could be 20 effected; and, further, the heat generated in the combustion of the carbonaceous material would fuse the metallic iron, which would then convert the phosphoric acid to its elemental condition and then absorb it.

25 The object of the invention herein is to so retard or lessen the combustion of the carbonaceous material as to afford opportunity for the combination of the carbon with the oxygen of the ore and to prevent the generation of such 30 a heat as will fuse the metallic iron, which in its molten condition will readily combine with the phosphorus.

In general terms, the invention consists in the process or method, all as more fully hereinafter described and claimed.

35 In the practice of my invention I take any suitable form of carbonaceous material—hard coal, or coke produced in the usual manner or by the combustion of fluids or by the distillation of oils, such as petroleum. The carbonaceous material is then broken up into small lumps and then ground up or reduced to about the size of coarse sand preparatory to mixing it with iron ore similarly prepared. These 40 small lumps or particles of carbonaceous material are then coated or covered with a thin lime or loam wash, which may be applied in any suitable manner—as, for example, pouring the wash over the carbonaceous material 45 or by immersing the latter in a bath of the wash. The carbonaceous material thus protected or coated is mixed with the broken or dis-

integrated ore in suitable proportions—about twenty-five to thirty-three per cent., more or less, by weight, of the ore. The mixed ore and 55 carbonaceous material are then charged into a suitable reverberatory furnace and there subjected to a sufficient degree of heat to liberate the oxygen from the ore and also to melt the matrix in which the iron is held. The 60 bottom of the reducing-furnace is formed first of a layer of comparatively large lumps of carbonaceous material and then with a layer of smaller lumps, and finally with a layer of fine material, which will fill the interstices between the lumps and form a smooth bed. The 65 material forming this bed is either coated with a wash of lime or loam prior to being placed in the furnace, or else a quantity of the wash is poured over the bed after being formed. 70 In lieu of forming the bottom of carbonaceous material, as above stated, unwashed graphite may be employed, if desired. The coating or wash will protect the carbonaceous material to such an extent as to prevent a rapid combustion thereof, and hence there will be a 75 slower generation of carbonic oxide. On account of this slow generation the carbonic oxide will be enabled to form a chemical union with the oxygen of the ore, thereby forming carbonic acid, whereas if the carbonaceous material were unprotected the oxygen would not be given off with sufficient rapidity to combine in proper proportions with the large volumes of carbonic oxide rapidly 80 evolved from the carbonaceous material.

The charge is heated to about a cherry-red heat and maintained thereat until the gangue is melted into a fluid slag and until the oxygen has been entirely removed, or practically so, 85 and the metallic iron brought into an adhesive state.

The fluid slag removes or takes up from the sponge a greater part of the impurities held therein, including phosphoric acid. When deoxidation has been effected and the metallic iron is in an adhesive condition, it is balled or worked up into masses of a suitable size, removed from the furnace, and immediately charged into an open-hearth furnace containing a bath of molten iron or steel. By balling up the iron and working it as free as possible from the slag, a comparatively pure mass of iron is obtained for subsequent working, and by 90 95 100

2

charging while hot it is immediately dissolved in the bath, and any impurities, including phosphorus, which it may contain are liberated and rise up into the slag before the 5 heat of the bath can so convert them as to permit of their absorption by the iron.

Any suitable material which will retard or lessen the combustion of the carbonaceous material may be employed in lieu of the lime or 10 loam to form the wash.

In some cases it is preferred to mingle the carbonaceous material and the ore and to charge them into the furnace before the wash or coating has become dry, thereby preventing 15 any loss of the ore and carbonaceous material in the form of dust.

I claim herein as my invention—

1. As a step in the art of manufacturing steel direct from ore, the herein-described process, which consists in intimately mixing the 20 ore with a carbonaceous material protected as

against rapid combustion by a coating of suitable material, and then subjecting the mixed ore and carbonaceous material to the action of a reducing-flame in a suitable furnace, substantially as set forth. 25

2. As a step in the art of manufacturing steel direct from ore, the herein-described process, which consists in intimately mixing the ore with a carbonaceous material protected by 30 a coating of lime as against rapid combustion, and then subjecting the mixed ore and carbonaceous material to the action of the reducing-flame in a suitable furnace, substantially as set forth. 35

In testimony whereof I have hereunto set my hand.

MATTHEW GRAFF.

Witnesses:

W. B. CORWIN,  
DARWIN S. WOLCOTT.